# EUROPEAN PATENT SPECIFICATION

(11) **EP 3 395 458 B1**
(45) Date of publication and mention of the grant of the patent: **18.08.2021**
(21) Application number: 16879417.0
(22) Date of filing: 23.12.2016
(51) Int. Cl.: C22C 23/02, C22F 1/06

(54) **MAGNESIUM ALLOY SHEET AND METHOD FOR MANUFACTURING SAME**
BLECH AUS MAGNESIUMLEGIERUNG UND VERFAHREN ZUR HERSTELLUNG DAVON
MATÉRIAU DE TÔLE D'ALLIAGE DE MAGNÉSIUM ET PROCÉDÉ DE FABRICATION ASSOCIÉ

(30) Priority: 23.12.2015 KR 20150185017; 24.12.2015 KR 20150186295
(43) Date of publication of application: 31.10.2018
(73) Proprietor: POSCO, Nam-gu Pohang-si, Gyeongsangbuk-do 37859 (KR)
(72) Inventor: PARK, Jun Ho, Pohang-si, Gyeongsangbuk-do 37859 (KR); KWON, Oh Duck, Pohang-si, Gyeongsangbuk-do 37859 (KR); LEE, Hyun Bom, Pohang-si, Gyeongsangbuk-do 37859 (KR); KiM, Jae Joong, Pohang-si, Gyeongsangbuk-do 37859 (KR)
(74) Representative: Potter Clarkson
(86) International application number: PCT/KR2016/015228
(87) International publication number: WO 2017/111550

(56) References cited:
- JP-A- 2009 007 606
- JP-A- 2010 229 467
- JP-A- 2011 074 461
- JP-A- 2011 179 075
- JP-A- 2011 184 726
- KR-A- 20150 065 418
- KR-B1- 101 078 308
- KR-B1- 101 481 909

## Description

### SAME

### [Technical Field]

The invention relates to a magnesium alloy sheet, and method for manufacturing thereof.

### [Background Art]

At present, the limitation of carbon dioxide emission and the importance of renewable energy are becoming the conversation topic in the international community and accordingly, lightweight alloys, which are a type of structural materials, are recognized as very attractive research fields.

In particular, magnesium is the lightest metal with a density of 1.744 g/cm³ and has various advantages such as vibration absorbing ability and electromagnetic shielding capability as compared with other structural materials such as aluminum and steel. Therefore related industry researches are being actively carried out to utilize magnesium.

Alloys comprising magnesium are currently being applied not only in the field of electronic devices but also in the field of vehicles, but they have fundamental problems in corrosion resistance, flame resistance, and formability, therefore there are limitations in expanding the application range.

Especially with regard to formability, magnesium is a HCP structure (Hexagonal Closed Packed Structure), and it does not exhibit an adequate slip system at room temperature, making it difficult to process. That is, a large amount of heat is required in magnesium processing, and this leads to an increase in cost.

On the other hand, among the magnesium alloys, the AZ system magnesium alloys comprise aluminum (Al) and zinc (Zn), which are inexpensive and yet commercially available magnesium alloys, securing adequate strength and ductility.

However, the physical properties mentioned above mean that it has an appropriate level among the magnesium alloys, and the strength is lower than that of aluminum (Al), which is competitive material.

Therefore, it is necessary to improve the physical properties such as low formability and strength of the AZ system magnesium alloy, but there is a lack of research in this area.

JP 2011 179075 A discloses a method of manufacturing a magnesium alloy sheet by adding 0.01 - 0.5 wt% Ca to a commercial Mg-AI-Zn-Mn-based alloy, hot rolling at a surface temperature of 450 - 566°C and annealing.

JP 2011 074461 A discloses a method of producing a similar alloy including steps of rough rolling the alloy in a reduction ratio of 40 - 60% at a temperature of 300 - 400°C and subsequently finish rolling in a lower reduction ratio and temperature.

JP 2011 184726 A discloses a method of producing a magnesium alloy sheet exhibiting cold formability equal to that of an aluminium alloy, comprising rolling a previously extrusion moulded alloy at a surface temperature of 490 - 566°C and at an angle that differs from the extrusion direction.

### [DISCLOSURE]

### [Technical Problem]

The present invention is intended to provide a method of manufacturing magnesium alloy sheet with improved strength and formability.

### [Technical Solution]

The invention is disclosed in the appended claims.

### [Advantageous Effects]

The center segregation which is likely to be generated in a conventional magnesium alloy sheet is avoided and the formability is improved in a magnesium alloy sheet according to an embodiment of the present invention.

In addition, according to an embodiment the present invention may provide a magnesium alloy sheet in which the texture of the magnesium alloy sheet is homogeneously dispersed, and the formability of which is improved.

In addition, according to another embodiment the present invention may provide a magnesium alloy sheet in which secondary phase particles of Al-Ca system are formed in a magnesium alloy sheet and strength is improved.

Methods for manufacturing a magnesium alloy sheet according to an embodiment of the present invention may provide a magnesium alloy sheet which is excellent in strength and formability by controlling the manufacturing process of a commercially available magnesium alloy. Because of this, it may be applied to appliances of vehicle or IT mobile devices in the future.

### [Description of the Drawings]

FIG. 1 is a schematic flowchart of part of a method of manufacturing a magnesium alloy sheet disclosed herein.
FIG. 2 is an image of scanning electron microscope (SEM) of the magnesium alloy sheet produced in Example 1.
FIG. 3 is an image of scanning electron microscope of the magnesium alloy sheet produced in Comparative Example 1.
FIG. 4 is an image of a Secondary Electron Microscopy of the magnesium alloy sheet produced in Example 1.
FIG. 5 is an image of a result of measuring the limiting dome height of the magnesium alloy sheet produced in Example 1.
FIG. 6 is a result of analysis of the crystal orientation by the XRD analyzer of the magnesium alloy sheet produced in Example 1.
FIG. 7 is a result of analysis of the crystal orientation by the XRD analyzer of the magnesium alloy sheet produced in Comparative Example 1.
FIG. 8 is an image of Electron Backscatter Diffraction (EBSD) of the magnesium alloy sheet produced in Example 1.
Fig. 9 is a result of EBSD analysis of the surface according to the reduction ratio in the skin pass process.
FIG. 10 shows the aggregate strength of the (0001) surface of Examples and Comparative Examples of the present invention.

### [Mode for Invention]

The first term, second and third term, etc. are used to describe various parts, components, regions, layers and/or sections, but are not limited thereto.

These terms are only used to distinguish any part, component, region, layer or section from other part, component, region, layer or section. Therefore, the first part, component, region, layer or section may be referred to as the second part, component, region, layer or section within the scope unless excluded from the scope of the present invention.

The terminology used herein is only to refer specific embodiments and is not intended to be limiting of the invention. The singular forms used herein comprise plural forms as well unless the phrases clearly indicate the opposite meaning. The meaning of the term "comprise" is to specify a particular feature, region, integer, step, operation, element and/or component, not to exclude presence or addition of other features, regions, integers, steps, operations, elements and/or components.

Although not defined differently, every term comprising technical and scientific terms used herein have the same meaning as commonly understood by those who is having ordinary knowledge of the technical field to which the present invention belongs. The commonly used predefined terms are further interpreted as having meanings consistent with the relevant technology literature and the present content and are not interpreted as ideal or very formal meanings unless otherwise defined.

In addition. % means weight% (wt%) unless otherwise referred.

Hereinafter, embodiments of the present invention will be described in detail with reference to the accompanying drawings so that those having ordinary knowledge in the art will easily carry out the invention. The present invention may, however, be implemented in several different forms and it is not limited to the embodiments described herein, but only by the scope of the appended claims.

The magnesium alloy sheet according to an embodiment of the present invention contains 2.7 to 5 wt% of Al, 0.75 to 1 wt% of Zn, 0.1 to 1 wt% of Ca, more than 0 wt% to 1 wt% of Mn and consist of the balance of Mg and inevitable impurities.

Hereinafter, the reason for limiting the numerical value of the component content in the embodiment of the present invention will be described.

First, aluminum (Al) improves the mechanical properties of the magnesium alloy sheet and castability of the molten metal. If Al is added too much, the castability may deteriorate rapidly, and if too little Al is added, the problem that mechanical properties deteriorate may occur. Therefore, the content range of Al may be adjusted within the range mentioned above.

Zinc (Zn) improves the mechanical properties of the magnesium alloy sheet. If too much Zn is added, a large number of surface defects and center segregation may be generated, leading to a problem of rapidly deteriorated castability, and if too little Zn is added, the problem that mechanical properties of magnesium alloy sheet deteriorate may occur. Therefore, the content range of Zn may be adjusted within the range mentioned above.

Calcium (Ca) gives flame resistance to the magnesium alloy sheet. If too much Ca is added, the fluidity of the molten metal is reduced, the castability becomes worse, and the center segregation made of the Al-Ca system intermetallic material is generated, which may cause a problem of deteriorating the formability of the magnesium alloy sheet, and if too little is added, the problem that the flame resistance is not sufficiently given may occur. Therefore, the content range of Ca may be adjusted within the range mentioned above. More specifically, Ca may be comprised 0.3 to 0.8 % (wt%).

Manganese (Mn) improves the mechanical properties of the magnesium alloy sheet material. If too much Mn is added, the problems that the heat emission is reduced and at the same time, uniform distribution control is difficult, may occur. Therefore, the content range of Mn may be adjusted within the above-mentioned range.

The magnesium alloy sheet alloy sheet according to an embodiment of the present disclosure may comprise Al-Ca secondary phase particles comprising 20 to 25% wt% of Al, 5 to 10% wt% of Ca and the balance of Mg. In general, when alloying by adding Al and Ca to magnesium, center segregation consisting of an Al-Ca intermetallic compound is generated which significantly reduces formability. On the other hand, the magnesium alloy sheet according to an embodiment of the present disclosure may improve formability by comprising Al-Ca secondary phase particles. The average particle diameter of the Al-Ca secondary phase particles may be 0.01 to 4 *µ*m. The formability may be further improved in the above-mentioned range. In addition, the Al-Ca secondary phase particles may comprise 5 to 15 particles per 100*µ*m² square of the magnesium alloy sheet material. By comprising Al-Ca secondary phase particles in the above-mentioned scope, the formability of the magnesium alloy sheet may be further improved. In order to obtain the above-mentioned Al-Ca secondary phase particles, the composition ranges of Al, Zn, Mn, and Ca, the temperature and time conditions during the homogenization heat treatment, the temperature and the rolling rate during warm rolling are precisely controlled.

The magnesium alloy sheet may comprise crystal grains and the average particle size of the crystal grains is 5 to 30 *µ*m. The formability may be further improved within the range mentioned above. In order to obtain crystal grains of the above-mentioned sizes, the composition scopes of Al, Zn, Mn, and Ca, the temperature and time conditions during the homogenization heat treatment, the temperature and the rolling rate during warm rolling are precisely controlled.

In addition, the limiting dome height of the magnesium alloy sheet according to the present invention is 7 mm or more. More specifically, it may be 8 mm or more, more specifically 8 to 10 mm.

In general, the limiting dome height is an index for evaluating the formability (especially, compressibility) of the material. The formability of the material is improved as the limiting dome height increases.

The limited range mentioned above is a significantly higher limiting dome height than in generally known magnesium alloy sheet, and is caused by an increase in the distribution of crystal grain orientation in magnesium alloy sheet.

In addition, the thickness of the magnesium alloy sheet according to an embodiment of the present disclosure may be 0.4 to 3 mm.

FIG. 1 schematically shows a flow chart of part of a method manufacturing a magnesium alloy sheet according to an embodiment of the present disclosure. The flow chart of a method manufacturing a magnesium alloy sheet of FIG. 1 is only to illustrate certain principles of the disclosure.

A method of manufacturing a magnesium alloy sheet as disclosed but not claimed herein comprises the steps of casting a molten metal containing 2.7 to 5 wt% of Al, 0.75 to 1 wt% of Zn, 0.1 to 1 wt% of Ca and more than 0 wt% to 1 wt% of Mn and the balance of Mg and inevitable impurities to produce a cast material (S10); subjecting the cast material to homogenization heat treatment (S20); and warm-rolling the cast material subjected to homogenization treatment (S30). In addition, if necessary, the manufacturing method of the magnesium alloy sheet may further comprise other steps.

First, in the step (S10), a molten metal containing 2.7 to 5 wt% of Al, 0.75 to 1 wt% of Zn, 0.1 to 1 wt% of Ca and more than 0 wt% to 1 wt% of Mn and consisting of the balance of Mg and inevitable impurities is cast to produce a cast material.

The reason for limiting the numerical value of the respective components is same as that described, therefore repeated descriptions will be omitted.

At this time, a method of casting the cast material may be die casting, strip casting, centrifugal casting, tilting casting, sand casting, direct chill casting or a combination thereof. More specifically, strip casting may be used.

More specifically, in the step of producing the cast material the reduction pressure may be 0.2 ton/mm² or more. More specifically, it may be 1 ton/mm² or more. More specifically, it may be 1 to 1.5 ton/mm² or more.

The cast material is produced by casting. At this time, when the cast material is coagulated and reduction pressure is simultaneously applied, the formability of the magnesium alloy sheet may be improved by adjusting the reduction pressure to the range mentioned above. In the step (S20), the cast material is subjected to homogenization heat treatment. At this time, the heat treatment condition is at a temperature of 350 to 500 °C for 1 to 28 hours. More specifically, it may be subjected to homogenization heat treatment for 18 to 28 hours. If the temperature is too low, the homogenization treatment cannot be properly performed, and there may occur a problem that beta phases such as Mg₁₇A₁₂ are not be employed at the base. If the temperature is too high, beta phases condensed in the cast material may melt, resulting in a fire or resulting in holes in the magnesium sheet. Therefore, it may be subjected to homogenization heat treatment within the temperature range described above.

In the step (S30), the homogenized cast material is warm-rolled. At this time, the temperature condition of the warm-rolling is at a temperature of 150 to 350 °C. If the temperature is too low, there may occur a problem generating a large amount of edge crack. If the temperature is too high, there may occur a problem being inappropriate for mass production. Therefore, warm-rolling may be within the above-mentioned temperature range.

The step of warm-rolling may be performed a plurality of times, and warm-rolling may be at a reduction ratio of 10 % to 30 % per time. By carrying out warm-rolling a plurality of times, finally the sheet may be rolled to a thin thickness of 0.4 mm.

The method as disclosed but not claimed may further comprise at least one step of intermediate annealing in the middle of a plurality of times of warm-rolling. The formability of the magnesium alloy sheet may be further improved by comprising the step of intermediate annealing. More specifically, the step of intermediate annealing may be carried out at a temperature of 300 to 500 °C for 1 to 10 hours. More specifically, it may be carried out at a temperature of 450 to 500 °C. The formability of the magnesium alloy sheet may be improved within the range mentioned above.

After the step of warm-rolling (S30), the sheet may further be subject to subsequent heat treatment. The formability of the magnesium alloy sheet may be improved by comprising the step of subjecting it to subsequent heat treatment. The step of subjecting to subsequent heat treatment may be carried out at a temperature of 300 to 500 °C for 1 to 10 hours. The formability of the magnesium alloy sheet may be further improved within the above-mentioned range.

A method for manufacturing a magnesium alloy sheet according to an embodiment of the present invention comprises the steps of preparing a master alloy comprising 2.7 wt% or more and 5 wt% or less of Al, 0.75 wt% or more and 1 wt% or less of Zn, 0.1 wt% or more and 0.7 wt% or less of Ca, more than 0 wt% and 1 wt% or less of Mn and the balance of inevitable impurities and magnesium, for a total of 100 wt%; casting the master alloy to produce a cast material; subjecting the cast material to homogenization heat treatment; warm-rolling the cast material subjected to homogenization heat treatment to produce a rolled material; subjecting the rolled material to subsequent heat treatment; and carrying out a skin pass on the rolled material subjected to subsequent heat treatment to produce a magnesium alloy sheet.

First, in the step of preparing a master alloy, that is not claimed herein, comprising 2.7 wt% or more and 5 wt% or less of Al, 0.75 wt% or more and 1 wt% or less of Zn, 0.1 wt% or more and 0.7 wt% or less of Ca, more than 0 wt% and 1 wt% or less of Mn and the balance of inevitable impurities and magnesium, for a total of 100 wt%, the master alloy may be commercially available AZ31 alloy, AL5083 alloy or a combination thereof. However, the disclosure is not limited thereto.

Next, the step of casting the master alloy to produce a cast material; is carried out.

More specifically, the master alloy may be dissolved to prepare the molten metal at the temperature range of 650 to 750 °C. Thereafter, the molten metal may be cast to produce a cast material. At this time, the thickness of the cast material may be 3 to 7 mm.

At this time, a method of casting the cast material may be die casting, strip casting, centrifugal casting, tilting casting, sand casting, direct chill casting or a combination thereof. More specifically, strip casting may be used. However, the method is not limited thereto.

In the step of producing the cast material, the reduction pressure may be 0.2 ton/mm² or more. More specifically, it may be 1 ton/mm² or more. More specifically, it may be 1 to 1.5 ton/mm² or more.

Thereafter, the step of subjecting the cast material to homogenization heat treatment is carried out.

More specifically, the step of subjecting the cast material to homogenization heat treatment may comprise the step of a first heat treatment at a temperature scope of 300 °C to 400°C; and the step of a second heat treatment at a temperature scope of 400 °C to 500 °C. More specifically, the step of first heat treatment at a temperature range of 300 °C to 400 °C may be carried out for 5 to 20 hours. In addition, the step of second heat treatment at a temperature range of 400 °C to 500 °C may be carried out for 5 to 20 hours.

By carrying out the first heat treatment at the temperature range mentioned above, the Mg-AI-Zn ternary system Pi-phase generated in the casting step may be removed. If the ternary system Pi-phase exists, the subsequent process may be adversely affected. In addition, the stress in the slab may be released by carrying out the second heat treatment step within the above-mentioned temperature range. Furthermore, it may actively induce the formation of recrystallization of the cast structure in the slab.

Thereafter, the step of warm-rolling the cast material subjected to homogenization heat treatment to produce the rolled material is carried out.

The heat-treated slab may be rolled to a thickness range of 0.4 to 3 mm through 1 to 15 times of rolling. In addition, the rolling may be carried out at a temperature of 150 °C to 350 °C.

More specifically, if the rolling temperature is less than 150 °C, it may induce a crack on the surface when rolling, and if it exceeds 350 °C, it may not be suitable for actual production facilities. Therefore, it may be rolled at 150 °C to 350 °C.

Next, the step of intermediate annealing the rolled material may be carried out. When it is rolled several times in the step of rolling, it may be subjected to heat treatment at the temperature range of 300 °C to 550 °C for 1 to 15 hours in the interval between successive passes. For example, it may be subjected to intermediate annealing once after rolling twice, and then rolled to a final target thickness. As another example, it may be rolled to the final target thickness by annealing once after rolling three times. More specifically, in the case where the rolled cast material is annealed in the above temperature range, the stress generated by rolling may be released. Therefore, it may be rolled several times up to the desired thickness of the cast material. Finally, the step of carrying out a skin pass on the rolled material subjected to subsequent heat treatment to produce a magnesium alloy sheet may be performed. More specifically, the skin pass is also known as skin pass rolling or temper rolling, which means that it removes a deformation pattern generated in a cold rolled steel sheet after heat treatment, and cold rolling with light pressure to improve the hardness.

Therefore, in an embodiment of the present invention, a skin pass is carried out once at a temperature range of 250 °C to 350 °C. More specifically, the magnesium alloy sheet manufactured by carrying out the skin pass is rolled at a reduction ratio of 6 to 15% with respect to the thickness of the rolled material. More specifically still, in the case of rolling under the conditions of temperature and pressure, the development of the texture, which is a weak base surface texture (0001) is reduced, so that formability may be obtained.

However, when the reduction ratio is 6 to 15 %, the yield strength may be 250 to 280 MPa, but value of the limiting dome height may be 7 to 8 mm since the texture is somewhat developed. This is because, as disclosed in FIG. 9, when rolling at a reduction ratio of 6 to 15%, a hardening occurs due to the double turning or dislocation. More specifically, when the reduction ratio is 2 to 6 %, the area fraction of the twinned crystal structure may be 5 % or less with respect to 100 % of the total area of the magnesium alloy sheet. More specifically, when the rolling is at the reduction ratio of 6 to 15 %, the area fraction of the twinned crystal structure is 5 to 20 % with respect to 100 % of the total area of the magnesium alloy sheet. In the image of the structure disclosed in FIG. 9, a black color means twinned crystal structure, and as described above the strength of the magnesium alloy sheet is maintained and the formability may be improved due to twinned crystal and dislocation.

Therefore, in the case of rolling with a reduction ratio greater than 15 %, the texture of the (0001) surface may be developed again and the formability may be lowered. This may be the same phenomenon that occurs when the temperature range during rolling is low. Therefore, the skin pass is carried out under the condition of temperature range and the reduction ratio according to the present invention.

In addition, the term "Limit Dome Height (LDH)" is an index for evaluating the formability of a sheet, particularly pressability, and may be measured by measuring the deformed height by applying a deformation to the specimen.

More specifically, the limit dome height (LDH) according to the present invention is the measured distance at which a punch moved until a disc-shaped specimen was fractured, that is, the height at which the specimen was deformed, by fixing a peripheral portion of a specimen having a diameter of 50 mm with a force of 10 KN and then applying a deformation at a rate of 5 to 10 mm/min using a spherical punch having a diameter of 20 mm at room temperature.

Hereinafter, preferred examples and comparative examples of the present invention will be described. However, the following examples are merely preferred examples of the present invention, and the present invention is not limited thereto.

### Non-claimed Example 1

A molten metal comprising 3.0 wt% of Al, 0.8 wt% of Zn, 0.6 wt% of Ca, 0.5 wt% of Mn and consisting of the balance of Mg and inevitable impurities was passed through between two cooling rolls having a reduction pressure of 1.2 ton/mm² to produce a magnesium cast material.

The magnesium alloy sheet having a final thickness of 0.7 mm was produced by carrying out subjecting the magnesium cast material to homogenization heat treatment at a temperature of 400 °C for 24 hours, warm-rolling at 250 °C at a reduction ratio of 15 %, intermediate annealing at 450 °C for 1 hour, and warm-rolling again at 250 °C at a reduction ratio of 15 %.

### Comparative example 1

A magnesium alloy sheet was produced in the same manner as in Example 1, except that 3.0 wt% of Al and 0.8 wt% of Zn were comprised.

### Test Example 1: Observation of microstructure that composes a magnesium alloy sheet.

The image of Scanning Electron Microscope (SEM) of the magnesium alloy sheet produced in Example 1 and Comparative Example 1 were shown in FIG. 2 and FIG. 4 respectively.

In the case of Example 1 (FIG. 2), the central segregation of the magnesium alloy sheet was hardly generated, whereas in the case of Comparative Example 1 (FIG. 3), it may be confirmed that a large amount of central segregation occurred. Such center segregation becomes a factor of being deteriorated the formability of the magnesium alloy sheet.

The image of Secondary Electron Microscopy of the magnesium alloy sheet produced in Example 1 was shown in FIG. 4.

The white dot portion in FIG. 4 is Al-Ca secondary phase particles. As a result of analyzing the white dot portion, analysis was made with 65.62 wt% of Mg, 24.61 wt% of Al, 8.75 wt% of Ca, 0.36 wt% of Mn and 0.66 wt% of Zn.

### Test Example 2: Measurement of limit dome height of a magnesium alloy sheet.

The limit dome height was determined by inserting each magnesium alloy sheet of the Examples and the Comparative examples between the upper die and the lower die and fixing the outer periphery of each specimen with a force of 5 kN and the press oil was used as the lubricant. Then, a spherical punch having a diameter of 30 mm was used to deform at a rate of 5 to 10 mm/min, the punch was inserted until each specimen was fractured and then it was performed when occurring such fracture in the manner of measuring of the deformation height of each specimen.

FIG. 5 is an image of a result of measuring the limit dome height of the magnesium alloy sheet produced in Example 1.

### Test Example 3: Analysis of crystal grain orientation.

The crystal orientation of each of the crystal grains of the magnesium alloy sheet produced in Example 1 and Comparative Example 1 confirmed by an XRD analyzer and was shown in FIG. 6 and FIG.7 respectively.

In the case of Example 1 (FIG. 6), contour lines are widely spread, and it may be confirmed that the crystal orientation of the crystal grains in the sheet are presented widely and variously. Therefore, it may be confirmed that the formability of Example 1 is excellent. On the other hand, in the case of Comparative Example 1 (FIG. 7), it may be confirmed that the (0001) peak is concentrated.

An image of the EBSD of Example 1 was taken and shown in FIG. 8. As shown in <b>, it may be known that the values of misorientation are evenly distributed in each of the crystal grains, and it may be confirmed that each of the crystal grains have various crystal orientations.

### Example 2

A master alloy comprising 3 % of Al, 1 % of Zn, 1 % of Ca, 0.3 % of Mn and the balance of magnesium and inevitable impurities was prepared.

The master alloy was cast to produce a cast material. The cast material was subjected to a first homogenization heat treatment at a temperature of 350 °C for 10 hours. The cast material subjected to a first homogenization heat treatment was subjected to a secondary homogenization heat treatment at a temperature of 450 °C for 10 hours. The cast material subjected to homogenization heat treatment was rolled to produce a rolled material. Thereafter, the rolled material was subjected to subsequent heat treatment at a temperature of 400 °C for 10 hours.

Finally, skin pass was carried out on the rolled material subjected to the subsequent heat treatment to produce the magnesium alloy sheet, the temperature and the reduction ratio of execution of the skin pass are shown in Table 1 below.

### Test Example 4: Test of Comparison of mechanical properties according to reduction ratio and temperature of skin pass.

**[Table 1]**

| | Rolling temperature (°C) | Reduction ratio(%) | Yield strength (MPa) | Maximum tensile strength (MPa) | Elongation (%) | Limit dome height (LDH, mm) |
|---|---|---|---|---|---|---|
| Example 2a | 250 | 5 | 202 | 257 | 22 | 8.1 |
| Example 2b | | 9 | 211 | 254 | 22 | 8.0 |
| Example 2c | | 15 | 252 | 272 | 16 | 7.3 |
| Comparative 2a | | 22 | 272 | 289 | 8.6 | 7.0 |
| Comparative 2b | 300 | X | 140 | 233 | 23 | 8-9 |
| Example 2d | | 7 | 203 | 253 | 22 | 8 |
| Example 2e | | 12 | 247 | 267 | 18 | 7.3 |
| Comparative 2c | | 17 | 247 | 272 | 10 | 7.3 |

As shown in Table 1, after carrying out the skin pass on the magnesium alloy sheet having the same component and composition, the yield strength was improved without greatly changing the formability. More specifically, the formability may be compared with the numerical values of the elongation and the limit dome height.

In addition, the formability was secured by minimizing the change in the aggregate strength, and the aggregate strength is as disclosed in FIG. 10 herein.

FIG. 10 shows the aggregate strength of (0001) surface of the Examples and Comparative Examples of the present invention.

As disclosed in FIG. 10, in the case of Comparative Examples 2a and 2c, it may be seen that the yield strength increases significantly as the change in the strength of the texture increases. However, it may be seen that the formability is somewhat reduced as the elongation is rapidly lowered.

Therefore, as disclosed in Table 1 and FIG. 10. It was confirmed that the present invention minimizes the change in strength of the texture to secure the formability.

### Non-claimed Example 3

As compared with Example 1, a magnesium alloy sheet material was produced under different conditions as disclosed in Table 2 below. As a result, the mechanical properties of the magnesium alloy sheet produced in Example 3 are disclosed in Table 3 below.

**[Table 2]**

| | Al content (wt%) | Ca content (wt%) | Cast roll reduction pressure (mm/ton) | Homogenization annealing time (hr) | Rolling temperature (°C) | Intermediate annealing temperature(°C) |
|---|---|---|---|---|---|---|
| Example 3a | 3 | 0.6 | 1.2 | 24 | 250 | 450 |
| Example 3b | 4 | 0.6 | 1.2 | 24 | 250 | 450 |
| Example 3c | 5 | 0.6 | 1 | 24 | 250 | 450 |
| Example 3d | 3 | 0.6 | 1.2 | 24 | 250 | 300 |
| Example 3e | 3 | 0.6 | 1.2 | 24 | 250 | 400 |
| Example 3f | 3 | 0.6 | 1.2 | 24 | 250 | 500 |
| Example 3g | 3 | 0.7 | 0.2 | 24 | 250 | 500 |
| Example 3h | 3 | 0.7 | 1.2 | 24 | 250 | 450 |
| Example 3i | 3 | 0.6 | 1 | 1 | 250 | 400 |
| Comparative 3a | 3 | 0.6 | 0.8 | 24 | 250 | None |
| Comparative 3b | 3 | 0.7 | 1.2 | 24 | 400 | 250 |
| Comparative 3c | 3 | 0.7 | 1 | 48 | 250 | 400 |
| Comparative 3d | 3 | 0.7 | 0.8 | 24 | 100 | 400 |

**[Table 3]**

| | Crystal grain size (*µ*m) | Sheet thickness (mm) | Yield strength (Mpa) | Limit dome height (LDH, mm) |
|---|---|---|---|---|
| Example 3a | 19 | 0.7 | 164 | 9.4 |
| Example 3b | 7 | 0.6 | 161 | 8.2 |
| Example 3c | 6 | 1 | 166 | 8.1 |
| Example 3d | 13 | 1 | 155 | 7.5 |
| Example 3e | 21 | 1 | 157 | 8 |
| Example 3f | 25 | 1 | 154 | 9.9 |
| Example 3g | 16 | 0.7 | 151 | 9 |
| Example 3h | 15 | 3 | 155 | 9.1 |
| Example 3i | 17 | 1 | 164 | 9 |
| Comparative 3a | 10 | 0.7 | 188 | 2.5 |
| Comparative 3b | 11 | 0.6 | 155 | 5 |
| Comparative 3c | 40 | 1.5 | 145 | 5.1 |
| Comparative 3d | 8 | 1 | 166 | 4.9 |

As a result, in the case of Comparative Examples 3a to 3d which did not satisfy the conditions of the homogenization annealing time, the rolling temperature and the intermediate annealing temperature, it was confirmed that the formability was inferior to the example of the present invention. In addition, the yield strength is also inferior to the example herein. In the case of comparative Example 3c, the size of the crystal grain was about 40*µ*m, which was relatively superior to the other comparative examples but was less than examples of the present invention.

The present invention is not limited to the above-mentioned examples or embodiments and may be manufactured in various forms, those who have ordinary knowledge of the technical field to which the present invention belongs may understand that it may be carried out in different and concrete forms without changing the technical idea or fundamental feature of the present invention as defined in the appended claims.

Therefore, the above-mentioned examples or embodiments are illustrative in all aspects and not limitative.

## Claims

1. A magnesium alloy sheet containing 2.7 to 5 wt% of Al, 0.75 to 1 wt% of Zn, 0.1 to 1 wt% of Ca and 1 wt% or less excluding 0 wt% of Mn and the balance of Mg and inevitable impurities, wherein the twin structure area fraction is 5 to 20 % with respect to 100% of the area of the magnesium alloy sheet, and wherein a maximum aggregate strength is 1 to 4 on the basis of the magnesium alloy sheet (0001) surface and wherein the limiting dome height (LDH) of the magnesium alloy sheet is 7 mm or more.

2. A magnesium alloy sheet according to Claim 1, wherein the yield strength of the magnesium alloy sheet is 170 to 300 MPa.

3. A method for manufacturing a magnesium alloy sheet according to Claim 1 or Claim 2 comprising the steps of preparing a master alloy comprising 2.7 wt% or more and 5 wt% or less of Al, 0.75 wt% or more and 1 wt% or less of Zn, 0.1 wt% or more and 1 wt% or less of Ca, more than 0 wt% and 1 wt% or less of Mn and the balance of inevitable impurities and magnesium, for a total of 100 wt%;
casting the master alloy to produce a cast material;
subjecting the cast material to homogenization heat treatment;
warm-rolling the cast material subjected to homogenization heat treatment to produce a rolled material;
subjecting the rolled material to subsequent heat treatment; and
carrying out a skin pass to the rolled material subjected to subsequent heat treatment to produce a magnesium alloy sheet,
wherein by the step of carrying out a skin pass to the rolled material subjected to subsequent heat treatment to produce a magnesium alloy sheet,
the produced magnesium alloy sheet is rolled at a reduction ratio of 6 to 15% with respect to the thickness of the rolled material;
wherein the step of carrying out a skin pass is carried out at a temperature in the range of 250°C to 350°C; and
wherein the step of subjecting the cast material to homogenization heat treatment comprises a first heat treatment step and a second heat treatment step.

4. The method for manufacturing a magnesium alloy sheet of Claim 3,
wherein the first heat treatment step comprises homogenization heat treatment at a temperature in the range of 300°C to 400°C; and
the second heat treatment step comprises homogenization heat treatment at a temperature in the range of 400°C to 500°C;
wherein the first heat treatment step at a temperature in the range of 300° to 400°C is carried out for 5 to 20 hours, and
wherein the second heat treatment step at a temperature in the range of 400°C to 500°C is carried out for 5 to 20 hours.

## Patentansprüche

1. Magnesiumlegierungsblech, das 2,7 bis 5 Gew.-% Al, 0,75 bis 1 Gew.-% Zn, 0,1 bis 1 Gew.-% Ca und höchstens 1 Gew.-% ausschließlich 0 Gew.-% Mn und den Rest Mg und unvermeidliche Verunreinigungen enthält, wobei der Doppelstrukturflächenanteil 5 bis 20 % hinsichtlich 100 % der Fläche des Magnesiumlegierungsblechs beträgt, und wobei eine maximale Gesamtfestigkeit 1 bis 4 auf der Basis der Magnesiumlegierungsblech-(0001)-Oberfläche beträgt und wobei die Grenzkuppelhöhe (limiting dome height - LDH) des Magnesiumlegierungsblechs wenigstens 7 mm beträgt.

2. Magnesiumlegierungsblech nach Anspruch 1, wobei die Streckgrenze des Magnesium legierungsblechs 170 bis 300 MPa beträgt.

3. Verfahren zum Erzeugen eines Magnesiumlegierungsblechs nach Anspruch 1 oder 2, umfassend die Schritte zum Herstellen einer Vorlegierung, umfassend wenigstens 2,7 Gew.-% und höchstens 5 Gew.-% Al, wenigstens 0,75 Gew.-% und höchstens 1 Gew.-% Zn, wenigstens 0,1 Gew.-% und höchstens 1 Gew.-% Ca, mehr als 0 Gew.-% und höchstens 1 Gew.-% Mn und den Rest unvermeidliche Verunreinigungen und Magnesium für insgesamt 100 Gew.-%;
Gießen der Vorlegierung, um ein Gussmaterial zu produzieren;
Unterziehen des Gussmaterials einer Homogenisierungswärmebehandlung;
Warmwalzen des Gussmaterials, das einer Homogenisierungswärmebehandlung unterzogen wird, um ein gewalztes Material zu produzieren;
Unterziehen des gewalzten Materials einer anschließenden Wärmebehandlung; und
Durchführen eines Dressierstichs an dem gewalzten Material, das einer anschließenden Wärmebehandlung unterzogen wird, um ein Magnesiumlegierungsblech zu produzieren,
wobei durch den Schritt des Durchführens eines Dressierstichs an dem gewalzten Material, das einer anschließenden Wärmebehandlung unterzogen wird, um ein Magnesiumlegierungsblech zu produzieren,
das hergestellte Magnesiumlegierungsblech mit einem Reduktionsverhältnis von 6 zu 15 % hinsichtlich der Dicke des gewalzten Materials gewalzt wird;
wobei der Schritt des Durchführens eines Dressierstichs bei einer Temperatur in dem Bereich von 250 °C bis 350 °C durchgeführt wird; und
wobei der Schritt des Unterziehens des Gussmaterials einer Homogenisierungswärmebehandlung einen ersten Wärmebehandlungsschritt und einen zweiten Wärmebehandlungsschritt umfasst.

4. Verfahren zum Erzeugen eines Magnesiumlegierungsblechs nach Anspruch 3,
wobei der erste Wärmebehandlungsschritt eine Homogenisierungswärmebehandlung bei einer Temperatur in dem Bereich von 300 °C bis 400 °C umfasst; und
wobei der zweite Wärmebehandlungsschritt eine Homogenisierungswärmebehandlung bei einer Temperatur in dem Bereich von 400 °C bis 500 °C umfasst;
wobei der erste Wärmebehandlungsschritt bei einer Temperatur in dem Bereich von 300 °C bis 400 °C 5 bis 20 Stunden lang durchgeführt wird, und
wobei der zweite Wärmebehandlungsschritt bei einer Temperatur in dem Bereich von 400 °C bis 500 °C 5 bis 20 Stunden lang durchgeführt wird.

## Revendications

1. Tôle d'alliage de magnésium contenant 2,7 à 5 % en poids d'AI, 0,75 à 1 % en poids de Zn, 0,1 à 1 % en poids de Ca et 1 % en poids ou moins à l'exclusion de 0 % en poids de Mn et le complément de Mg et d'impuretés inévitables, la fraction de zone de structure jumelle étant de 5 à 20 % par rapport à 100 % de la zone de la tôle d'alliage de magnésium, et la force maximale d'agrégat étant de 1 à 4 sur la base de la surface de la tôle d'alliage de magnésium (0001) et la hauteur limitante du dôme (LDH) de la tôle d'alliage de magnésium étant de 7 mm ou plus.

2. Tôle d'alliage de magnésium selon la revendication 1, dans laquelle la limite d'élasticité de la tôle d'alliage de magnésium est de 170 à 300 MPa.

3. Procédé de fabrication d'une tôle d'alliage de magnésium selon la revendication 1 ou la revendication 2, comprenant les étapes de préparation d'un alliage mère comprenant 2,7 % en poids ou plus et 5 % en poids ou moins d'AI, 0,75 % en poids ou plus et 1 % en poids ou moins de Zn, 0,1 % en poids ou plus et 1 % en poids ou moins de Ca, plus de 0 % en poids et 1 % en poids ou moins de Mn et le complément d'impuretés inévitables et de magnésium, pour un total de 100 % en poids ;
la coulée de l'alliage mère pour produire un matériau coulé ;
la soumission du matériau coulé à un traitement thermique d'homogénéisation ;
le laminage à chaud du matériau coulé soumis à un traitement thermique d'homogénéisation pour produire un matériau laminé ;
la soumission du matériau laminé à un traitement thermique ultérieur ; et
le fait d'effectuer un écrouissage du matériau laminé soumis à un traitement thermique ultérieur pour produire une tôle d'alliage de magnésium,
dans lequel, lors de l'étape consistant à effectuer un écrouissage du matériau laminé soumis à un traitement thermique ultérieur pour produire une tôle d'alliage de magnésium,
la tôle d'alliage de magnésium produite est laminée à un rapport de réduction de 6 à 15 % par rapport à l'épaisseur du matériau laminé ;
dans lequel l'étape consistant à effectuer un écrouissage est effectuée à une température comprise dans la plage de 250 °C à 350 °C; et
dans lequel l'étape consistant à soumettre le matériau coulé à un traitement thermique d'homogénéisation comprend une première étape de traitement thermique et une seconde étape de traitement thermique.

4. Procédé de fabrication d'une tôle d'alliage de magnésium selon la revendication 3,
dans lequel la première étape de traitement thermique comprend un traitement thermique d'homogénéisation à une température comprise dans la plage de 300 °C à 400 °C ; et
la seconde étape de traitement thermique comprend un traitement thermique d'homogénéisation à une température comprise dans la plage de 400 °C à 500 °C ;
dans lequel la première étape de traitement thermique à une température comprise dans la plage de 300 °C à 400 °C est effectuée pendant 5 à 20 heures, et
dans lequel la seconde étape de traitement thermique à une température comprise dans la plage de 400 °C à 500 °C est effectuée pendant 5 à 20 heures.
